

## UNITED STATES PATENT OFFICE

2,414,199

## FROTH FLOTATION OF NONSULFIDE ORES

Gregoire Gutzeit, Westport, Conn.

No Drawing. Application September 8, 1943,  
Serial No. 501,563

4 Claims. (Cl. 209—166)

1

The present invention relates to flotation, and more particularly to the recovery of desired minerals from ores containing the same by application of froth flotation methods.

It is an object of the invention to provide an improved flotation procedure in which, through the application of a chemical principle not heretofore recognized in the flotation art, unwanted gangue materials are deactivated or depressed and thereby largely eliminated from the concentrate of desired minerals, thus improving the grade of the concentrate to a marked degree. It is also an object of the invention to provide an improved flotation procedure in which, through the application of the same chemical principle, a selective separation can be made between two valuable minerals.

Froth-flotation is roughly based on the fact that the surface of a given mineral to be recovered can be rendered, by the action of so-called collectors, more or less water repellent, i. e. aero-phil, and a mineral-air complex, the specific gravity of which is lower than that of the pulp, is thus formed with the air bubbles introduced into the pulp. The binding of the collector to the mineral surface by chemical reaction, chemo-adsorption, adsorption, etc., is due to electrostatic forces, i. e. unsaturated valences, both of the collector itself and of the said surfaces.

It is the custom to speak about "differential" flotation, only in the case of polymetallic concentration, but most of the usual monometallic flotation are also differential ones, as the gangue has to be prevented from floating together with the wanted mineral. If the used collector has a tendency to be adsorbed by the gangue (which is particularly the case of paraffinic oils, fatty acids, fatty alcohols, sulfated and sulfonated alkyl-compounds, etc., chiefly used in the flotation of metallic oxide ores and non-metallic ores), the latter must be "depressed." Roughly, depression consists in the action of preventing the binding of the collecting reagent to the surface of a certain mineral which is not wanted in the concentrate. In the case of monometallic flotation, the gangue minerals which are mostly quartz and silicates, but which may also be carbonates of the alkaline earths, must be depressed. In the case of polymetallic flotation, the gangue, together with other valuable metallic minerals, have to be kept from floating, or a single mineral has to be collected, while others are prevented from concentrating in the froth.

Although the usual gangue minerals (with a few exceptions like talc, graphite, etc.) when pure, are naturally more hydrophilic than the valuable metal-bearing ones, they are easily floated after activation with metallic cations. Thus, quartz and most other silicates may be activated by very small amounts of iron, copper, zinc, lead, nickel, tin, titanium, barium, and some other

2

cations, and calcite by barium, copper, iron, and lead salts when floated with fatty acid or fatty alcohol collectors at pH values varying with each activating ion. Since in almost every pulp there are soluble metallic salts present such as dissolved iron from the ball-mill, or copper, zinc, or iron sulfates from the oxidization of sulfide-minerals, the gangue is always more or less activated and tends to concentrate in the flotation froth. This is particularly true when anion active high molecular aliphatic acids and alcohols, or their derivatives are used as collectors. In order to keep the gangue from floating, it is usual to add alkalies such as sodium carbonate, sodium hydroxide and the like, or sodium silicate, or acids. Alkalies form easily wettable hydroxides with the activating cations and increase the hydrophilic character of quartz and the silicates by their tendency to form soluble alkali-silicates. Sodium silicate forms insoluble metallic-silicates and hydrated metallic silica gels with the activating cations. The acidification of the pulp tends to replace the adsorbed metallic cations by more positive hydrogen ions which are hydrophilic, and increases the solubility of certain minerals. In addition to the effect of the alkalies, the use of alkali cyanide for the depression of the gangue has been proposed. Cyanide forms soluble complexes with some activating heavy metal cations, removing them by means of this reaction from the gangue material.

It will be seen, therefore, that in the flotation of ores, chemical and physical control is directed, firstly, toward increasing the flotability of the wanted minerals and, secondly, toward minimizing any flotation tendency exhibited by the unwanted gangue minerals contained in the admixture.

The present invention has the second of these objectives in view and, for the accomplishment of the same, it proposes to add to the flotation pulp relatively small amounts of certain organic compounds, which will be described presently, that react with the extraneous metal cations present so as to prevent the activation and flotation of unwanted gangue minerals by the agency of such cations.

Broadly, the invention embraces the addition to a flotation pulp of an organic compound able to form very stable, water soluble, or insoluble, but hydrophilic, inner complexes (chelate compounds) with the extraneous metallic cations in solution or adsorbed on the mineral particles, whereby such ions are prevented or inhibited from exerting an activating effect on the gangue particles.

Activation of the gangue minerals by metallic ions has been proved the fundamental condition for their flotation with cationic collectors of the fatty acid type. A. M. Gaudin and Alfonso Rizo Pat'n, T. P. No. 1453, A. I. M. E., February 1942,

have studied the mechanism of quartz activation by barium salts using oleic acid as collector, and demonstrated that effective quartz flotation only takes place in alkaline pulp, after abstraction of barium ions, the optimum ratio of collector to activating ion being 1:1. The mechanism of this cation adsorption is postulated to be a result of the ruptured bonds on the quartz surface, and the maximum barium-ion adsorption is calculated to be 1.7 micromol.

Following L. Kraeber and A. Boppel ("Metall & Erz," XXXI, 19), the cations listed below will definitely activate quartz within the indicated pH range:

| Cation            | pH range |
|-------------------|----------|
| Cu <sup>++</sup>  | 6.0-10.0 |
| Mg <sup>++</sup>  | 9.5-12.0 |
| Ca <sup>++</sup>  | 9.5-14.0 |
| Cd <sup>++</sup>  | 7.0-10.0 |
| Ba <sup>++</sup>  | 9.5-14.0 |
| Tl <sup>+++</sup> | 2.0-6.5  |
| Zn <sup>++</sup>  | 3.0-7.5  |
| Sn <sup>++</sup>  | 5.0-10.0 |
| Pb <sup>++</sup>  | 3.0-8.0  |
| Th <sup>+++</sup> |          |
| Cr <sup>+++</sup> | 3.0-7.5  |
| Fe <sup>+++</sup> | 6.5-10.5 |
| Ni <sup>++</sup>  |          |

The ions Li<sup>+</sup>, Ce<sup>++++</sup>, Zn<sup>++</sup> (ph 7-9), Al<sup>+++</sup> are less effective. W. Halbich proved that calcite and baryte are also activated by Ca<sup>++</sup>, Cu<sup>++</sup>, Pb<sup>++</sup>, Ba<sup>++</sup>, Fe<sup>+++</sup>, Al<sup>+++</sup>, when floated with higher alcohol sulfates.

As can be seen, common ions like Fe<sup>+++</sup>, Ca<sup>++</sup>, Mg<sup>++</sup>, almost always present in a flotation pulp, tend to activate the gangue minerals when fatty acids, alcohols or derivatives thereof (soaps, sulfonates, sulfates, phosphates, amine salts, etc.) are used as collectors.

Generally speaking, theretofore the flotation of non-sulfide ores (so called "non-metallics") has been performed with collectors which are mainly fatty acids, higher aliphatic alcohols, or derivatives thereof. These collectors, unlike for example, the xanthates used in the flotation of sulphides, are not very specific but have marked tendency to float the whole crude ore comprising the gangue (provided activation took place). As the aim of flotation is selective separation between the valuable mineral and the gangue, the latter has to be depressed.

As stated above, silica, the silicates, baryte and many light metal carbonates will not bind the fatty acid compounds chemically by themselves, but only by the intervention of adsorbed cations. If these extraneous activating cations can be rendered harmless by a chemical which will tie them up and remove them as an active factor in the process, the gangue minerals will exhibit no tendency to contaminate the concentrate. As the binding of the cation in an undissociable inner complex is quite complete, the proposed aim is fulfilled by the use of organic reagents able to form such complex compounds. However, at the same time, all excess cations are satisfied and yielded into an undissociable complex whereby readorption of the cations by the gangue is precluded.

In the field of selective flotation, the present invention makes possible the specific depression of one or several minerals, by addition of an excess (over 0.25 kg./t.) of the organic compounds to be described, for reacting with the cations at the surface of the mineral so as to prevent flotation by rendering said surface hydrophilic or water-avid.

Broadly, this second application of the invention embraces the addition to a flotation pulp of an organic compound able to form very stable, water soluble or insoluble but hydrophilic inner complexes (chelate compounds) with the metallic cations of one of the minerals, whereby such minerals are prevented from being reacted upon by the collector, and thus inhibited from concentrating in the flotation froth. It is very probable that even normal collection of, say, chalcocite (copper sulfide) is due to the presence of adsorbed copper ions on the surface of the mineral (auto-activation). But even if this theory is not generally admitted, the formation of a hydrophilic complex with the metal atoms of the lattice would cause depression.

According to the accepted theory of ionization, soluble salts are dissociated to a greater or lesser extent into their respective positively charged cations and negatively charged anions, thus:



Furthermore, these elements are in a state of equilibrium and any change in the concentration of molecular (left) or ionic (right) components results in more or less dissociation, depending upon the direction of displacement.

The Cu<sup>++</sup> ions with their two positive, elementary charges are thus in a position not only to bind anions with an opposite charge and so to form new compounds by the simple process of stoichiometric chemical reaction (by electrovalence), but also to neutralize (by coordination valence) the charge which exists on dipolar compounds, that is, molecules possessing an unbalanced or asymmetric electric field. In the former case a new ionic copper compound is formed; in the latter case a neutral structure known as a complex is formed, in which the copper, as such, possesses a minimum of chemical activity.

While Cu<sup>++</sup>, or other metallic ions, in solution are therefore normally able to chemically combine with, or be adsorbed at the surface of the gangue minerals, the presence of such molecular group as is mentioned above causes these same ions to be withdrawn from solution into non-reacting complexes where they become relatively harmless, thus:



It is well known that in the blue solution formed, the copper is tied up in the complex ion (Cu(NH<sub>3</sub>)<sub>4</sub>)<sup>++</sup> which is relatively stable and only slightly ionized as compared with copper chloride itself. Nevertheless, a slight dissociation of this complex cation does occur, thus:



as proved by the fact that the Cu<sup>++</sup> can be precipitated by H<sub>2</sub>S. Instead of using inorganic dipolar molecules such as NH<sub>3</sub> in order to bind up the actually or potentially activating cations, this invention is based upon the principle that dissociated metallic ions in solution in the pulp liquid, or adsorbed on the gangue particles, may be caused to form much more stable, undissociable, water soluble or insoluble, but hydrophilic, inner complexes with specific organic chemicals, which will be set forth hereinafter, which are added to the pulp.

These specific organic reagents must possess in their molecule certain groups capable of uniting with metals through the replacement of the acidic hydrogen, the metal in the resultant compounds being held in position by a primary or

electro-valence, and, on the other hand, other groups being capable of combining with metals through the coordination bond, that is, without the replacement of hydrogen. If these two functional groups are both attached to one single organic radical in the proper relative position such as to satisfy the Baeyer strain theory, a cyclic structure will be formed which is known as an inner complex or chelate compound. The metal atom in these four, five or six membered rings is most frequently attached to a nitrogen, oxygen or a sulfur atom by electrovalence (salt formation), and it completes the cycle through coordinate valence linking it to another functional group containing nitrogen, oxygen or sulfur.

The conception "inner complex" may be defined for the purpose of this specification as a cyclic chemical structure containing an inorganic cation (or positively charged metal ion) that is bound simultaneously to several atoms in a single organic molecule, on the one hand by means of the ordinary valence bonds, or electron exchange; on the other hand through the action of an electric field which satisfies the secondary valences, the relative position of the salt- and the complex-forming groups being such that a four-, five- or six-membered ring is formed; and the characteristic property of such a compound is that the positive ion referred to is not in a condition, on account of the completeness of the bonding described, to enter into any normal chemical reaction involving ionic exchange or metathesis.

For example, the copper cation form normal dissociable salts with almost every water-soluble organic acid like acetic acid, thus



But, if instead of acetic acid, the amino derivative of the same (amino-acetic acid or glycocoll) is used, an inner complex results from the combination of the cation and the amino acid (copper glycine) thus:



This compound (complex copper glyconate) is soluble, but the copper atom is bound in such a complete manner that no more dissociation is possible. As a result, no measurable free  $\text{Cu}^{++}$  ions can be detected in the solution, no reaction occurs with  $\text{H}_2\text{S}$ , carbonates, caustic or even ammonia, and the solution of the complex shows practically no electrical conductivity.

This class of organic chemicals outlined above is used as reagents in inorganic analysis (especially in the spot test method), for they are or may be rendered specific toward certain cations. Some of them have also been proposed as flotation collectors, although mostly without a complete understanding of the fundamentals involved; for this last purpose they must form insoluble, hydrophobic coatings, i. e. an oriented water-repellent film, on the surface of the mineral particle. But, in order to fulfill the aim of deactivating or depressing the gangue by removal of the free or adsorbed metallic ions acting as actual or potential activators according to the present invention, the formed inner complexes or chelate compounds with said cations have to be water soluble or hydrophilic.

Thus, the present invention discloses the use of organic compounds capable of forming specific soluble or hydrophilic inner complexes with metallic ions in solution or adsorbed on the mineral particles, and thereby preventing such ions from exerting an activating influence on the gangue.

In addition to these general conditions required to form a cyclic chelate compound, the latter must be water soluble or hydrophilic in order to fulfill the desired purpose. The structural features promoting water solubility or hydrophilic character for an organic compound are not yet completely understood (Refer, in H. Gilman, "Organic Chemistry," John Wiley and Sons, Inc., New York, N. Y., 1938, the chapter: "Constitution and physical properties of organic compounds," by Wallace R. Brode and John A. Leermakers). Nevertheless, the following facts may help to clarify the relation between constitution and water affinity:

Water solubility is not merely a physical, but rather a chemical phenomenon, which depends upon the ability of the solute to bind dipolar water molecules (dipole moment of water  $\mu = 1.84 \cdot 10^{-18}$  e. s.). Hydrophilic, as will be shown, is closely related to solubility.

The similarity between the dissolved material and the molecules of the solvent appear to be very important to the whole problem of solution.

Because the combining power of the metal atom in a chelate compound is saturated by bonds and complex linkages with several atoms of the same organic molecule, inner complexes are mostly non-electrolytes and the attraction of water molecules (consequently, the hydration and the solubility) is inhibited as well as the dissociation. Thus, anthranilic acid (o-aminobenzoic acid) has a solubility of 230 grs. in 100 cc. of water at 107.8° C., while its cobalt complex is practically insoluble in boiling water.

Therefore, in addition to the structure required for the formation of a chelate compound (i. e., salt-forming group, complex-forming group and steric disposition allowing the closure of a four-, five- or six-membered ring), the organic depressing reagents, in order to yield soluble or hydrophilic inner complexes, ought to have additional features which will promote the hydration, i. e. groups tending to bind water molecules (or an electric field due to distortion having the same effect).

Groups which promote affinity towards water molecules for an organic compound are, for example, the amino, the carboxyl functions. (In the alkanes series, the amino group is generally more active than the carboxyl group, and the latter more active than the hydroxyl group.) But, in addition to the presence of these hydration centers, two other factors play an important role: (a) the balance between the polar (hydrophilic) function and the non-polar (hydrophobic) hydrocarbon radical; (b) the configuration of the molecule.

As a broad rule, it may be pointed out that each of the following structural features will impart water solubility or hydrophilicity to an inner complex:

Firstly, the chelate compound (aliphatic or aromatic) must have at least one free group containing one or both of the elements composing the water molecule (O and H). This is particularly the case for the hydroxy- and carboxyl-group, and, to a lesser extent, of the aldehyde and carbonyl-group. It shall be noted that the replacement of the oxygen atom by sulfur will result

in the formation of less soluble or insoluble complexes. As already pointed out, the length of the individual carbon chains of the radical in the aliphatic series must not overbalance the lyophilic function (i. e. contain, for example, less than 7 carbon atoms for a hydroxyl group, and less than 8 carbon atoms for a carboxyl group in the n-alkane series).

The configuration plays an important role, particularly in the aromatic series. Thus:

| Compound            | Solubility grs. in 100 grs. H <sub>2</sub> O |                        |
|---------------------|----------------------------------------------|------------------------|
|                     | Cold water                                   | Hot water              |
| o-Aminobenzoic acid | 0.341 <sup>4</sup>                           | 230.0 <sup>107.8</sup> |
| m-Aminobenzoic acid | 0.591 <sup>5</sup>                           | 24.8 <sup>105.2</sup>  |
| p-Aminobenzoic acid | 0.349.6                                      | 42.8 <sup>109.3</sup>  |

The above observations concerning structure 20 hold true for all the following points.

Secondly, the chelate compounds containing free inorganic acid radicals like sulfo-, phospho-, arseno-radicals, and the hydrochlorides of aromatic bases, etc., are generally soluble or hydrophilic. This is particularly the case for the aromatic sulfonates.

Thirdly, the trivalent nitrogen atom of amino groups (and heterocyclic compounds) promotes the solubility to an even higher degree than the 30 hydroxyl function.

Thus, n-butane is slightly soluble in water (15 cc. at 17° C. and 772 mm. pressure in 100 gr. water); 7.9 gr. n-butyl alcohol (butanol 1) dissolve in 100 gr. water at 20° C.; 5.62 gr. n-butylamine dissolve in 100 gr. water at -1° C.; while n-butylamine is completely miscible with water (solubility ∞). Acetic acid is completely miscible with water. Esterification of the carboxyl group gives insoluble compounds. But the introduction of an amino-group in an acetic ester brings back the solubility. Substitution of the hydrogen atoms of the NH<sub>2</sub> group decreases the solubility in simple (monofunctional) compounds, but increases this property in amino-acids.

#### EXAMPLE

(a)

| Compound      | Formula                                          | Solubility grs. in 100 grs. H <sub>2</sub> O | Dipole moment MX10 <sup>-18</sup> es. |
|---------------|--------------------------------------------------|----------------------------------------------|---------------------------------------|
| Ethylamine    | C <sub>2</sub> H <sub>5</sub> NH <sub>2</sub>    | ∞                                            | +1.31                                 |
| Diethylamine  | (C <sub>2</sub> H <sub>5</sub> ) <sub>2</sub> NH | 81.5 <sup>44</sup>                           | +0.94                                 |
| Triethylamine | (C <sub>2</sub> H <sub>5</sub> ) <sub>3</sub> N  | 1.5 <sup>20</sup>                            | +0.76                                 |

(b)

| Compound                       | Formula                                                                        | Solubility               |
|--------------------------------|--------------------------------------------------------------------------------|--------------------------|
| Amino acetic acid              | H <sub>2</sub> C—COOH<br>NH <sub>2</sub>                                       | 1 gr. in 4.3 gr./15° C.  |
| Acetic acid monoethylamine     | H <sub>2</sub> C—COOH<br>NH(C <sub>2</sub> H <sub>5</sub> )                    | Very soluble.            |
| Acetic acid diethylamine       | H <sub>2</sub> C—COOH<br>N(C <sub>2</sub> H <sub>5</sub> ) <sub>2</sub>        | Hygroscopic.             |
| α-Amino caproic acid           | NH <sub>2</sub><br>CH <sub>3</sub> (CH <sub>2</sub> ) <sub>5</sub> CHCOOH      | 1 gr. in 48.8 gr./12° C. |
| Caproic acid α-monomethylamine | CH <sub>3</sub> (CH <sub>2</sub> ) <sub>5</sub> CHCOOH<br>NH(CH <sub>3</sub> ) | 1 gr. in 9.8 gr./13° C.  |

It should be noted that, in α-amino acids, esterification of the carboxyl group increases the solubility. This is due to the fact that, in the free acids, the ionizable hydrogen is linked by a secondary valence to the nitrogen (of the amino function), thus blocking a coordination center for water molecules. Esterification liberates the amino group.

#### EXAMPLE

| Aminoacetic acid                                        | Aminoacetic acid ethyl ester                                       |
|---------------------------------------------------------|--------------------------------------------------------------------|
| $\text{CH}_2\text{—COOH}$<br>H <sub>2</sub> N—<br> <br> | $\text{CH}_2\text{COOC}_2\text{H}_5$<br>H <sub>2</sub> N—<br> <br> |

Soluble 1 gr. in 4.5 grs. water  
Miscible with water

A heterocyclic nitrogen atom, even acting as a center of coordination (complex forming group) yields soluble complexes if it belongs to a single ring (pyridine radical). Thus, α-picolinic acid



forms colored, soluble iron (Fe<sup>++</sup>) complexes, (as well as a silver complex), while the complexes of 8-oxyquinoline or α-quinaldic acid are generally insoluble.

Fourthly, if the lyophilic groups as mentioned above, especially the carboxyl and amino (primary, secondary or tertiary) functions, acting at the same time as salt-forming and complex-forming functions, overbalance the radical (i. e., the individual carbon chains) in a compound of the aliphatic series, the complex will be soluble even if no supplemental free lyophilic group is present. This is the case when no more than 40 4 carbon atoms are attached to the reactive grouping.

As shown above, the amino group (primary, secondary or tertiary) and the carboxyl group are very powerful solubility-promoting functions. On the other hand, the hydrogen of the carboxyl 45 group is easily dissociable (salt-forming group), while the nitrogen of the amino function and of heterocyclic N-compounds is one of the most active centers of coordination (complex-forming group). Therefore, organic compounds with one 50 amino nitrogen in alpha or beta position to one carboxyl group, and at least one additional amino or carboxyl group to impart water solubility, i. e. polycarboxylic amino acids, monocarboxylic polyamino acids, and polycarboxylic polyamino acids, 55 in which one amino group is in 1 or 2 position to one carboxyl function, will yield soluble or

hydrophilic inner complexes, and thus are excellent organic flotation depressants, through the binding of gangue activating cations into cyclic chelates.

These organic depressants, which are the specific subject of the present invention, have the following structural characteristics:

thetic compounds, and can be produced following U. S. P. 2,130,505 of September 20, 1938, (Ferdinand Münz, assignor to General Aniline Works, Inc., New York, N. Y.). The tetra acetic acid derivative (sodium salt) of ethylene diamine is manufactured by the General Dyestuff Corporation, 435 Hudson Street, New York, N. Y.,

| Class of compounds               | Salt-forming group | Complex-forming group                      | Example of reactive grouping                                                                                                                                                                                                                                                                                                                                                                                                                                                                                                                                                                                                                                                                                                                                                                                        | Hydrophilic group                                       | Examples                                                                                                                                                                                                                                                                                                                                                                                                                                                                                                                                                                                                                                                                                                                                                                                                                                                                                                                        |
|----------------------------------|--------------------|--------------------------------------------|---------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|---------------------------------------------------------|---------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|
| Monoamino poly-carboxylic acids. | $-\text{COOH}$     | $-\text{NH}_2, =\text{NH}, \text{N}\equiv$ | $\begin{array}{c} \text{O} \quad \text{H} \\ \parallel \quad   \\ \text{C} - \text{C} - \\   \quad   \\ \text{OH} \quad \text{NH}_2 \end{array}$<br>$\begin{array}{c} \text{H}_2 \quad \text{H} \\    \quad   \\ \text{C} - \text{C} - \text{C} \\   \quad   \\ \text{OH} \quad \text{NH}_2 \end{array}$<br>$\begin{array}{c} \text{HN} \quad \parallel \\   \quad \text{C} - \text{C} = \text{O} \\   \quad \text{OH} \end{array}$<br>$\begin{array}{c} \text{C} - \text{N} = \text{C} \\ \parallel \\ \text{C} - \text{OH} \\   \\ \text{O} \end{array}$<br>$\begin{array}{c} \text{H} \\   \\ \text{C} - \text{N} - \text{O} - \\   \\ \text{C} - \text{OH} \\   \\ \text{O} \end{array}$<br>$\begin{array}{c} \parallel \\ \text{C} - \text{N} = \text{C} \\ \text{HO} - \text{C} \\   \\ \text{O} \end{array}$ | $-\text{COOH}$                                          | Aspartic acid (aminosuccinic acid)<br>$\text{HO}_2\text{CCH}_2\text{CH}(\text{NH}_2)\text{CO}_2\text{H}$<br><br>Glutamic acid<br>$\text{HO}_2\text{C}(\text{CH}_2)_2\text{CH}(\text{NH}_2)\text{CO}_2\text{H}$<br><br>Iminodiacetic acid<br>$\text{CH}_3\text{CO}_2\text{H}$<br>$\begin{array}{c} \text{HN} \\   \\ \text{CH}_3\text{CO}_2\text{H} \end{array}$<br><br>Chelidamic acid (4 hydroxypyridine-2,6-dicarboxylic acid)<br>$\text{HO} \quad \text{OH}$<br>$\text{HO}_2\text{C} - \text{C} = \text{N} - \text{C} - \text{CO}_2\text{H} \rightleftharpoons \text{HO}_2\text{C} - \text{C} = \text{O} - \text{C} - \text{CO}_2\text{H}$<br><br>Pyridine dicarboxylic acids 2,3 quinolinic- 2,4 lutidinic-<br>2,6 dipicolinic; 2,5 isocinchomeric acids<br>$\begin{array}{c} \text{H} \\   \\ \text{C} \\    \\ \text{HC} \quad \text{C} - \text{COOH} \\   \quad   \\ \text{HC} \quad \text{C} - \text{COOH} \end{array}$ |
| Polyamino mono-carboxylic acids. | $-\text{COOH}$     | $-\text{NH}_2, =\text{NH}, \text{N}\equiv$ | $\begin{array}{c} \text{H} \\   \\ -\text{O} - \text{C} = \text{O} \\   \\ \text{H}_2\text{N} \quad \text{OH} \end{array}$<br>$\begin{array}{c} \text{H} \quad \text{H}_2 \\    \quad   \\ -\text{N} - \text{C} - \text{C} = \text{O} \\   \\ \text{OH} \end{array}$                                                                                                                                                                                                                                                                                                                                                                                                                                                                                                                                                | $-\text{NH}_2, =\text{NH}, \text{N}\equiv$              | Ornithine $\alpha, \delta$ diaminovaleric acid)<br>$\text{H}_2\text{N}(\text{CH}_2)_4\text{CH}(\text{NH}_2)\text{CO}_2\text{H}$<br><br>Arginine ( $\alpha$ amino- $\beta$ -guanidylvaleric acid)<br>$\text{H}_2\text{N}(\text{NH})\text{NH}(\text{CH}_2)_4\text{CH}(\text{NH}_2)\text{CO}_2\text{H}$<br><br>Guanidino acetic acid<br>$\text{H}_2\text{N}-\text{C}(\text{=NH})\text{NH}-\text{CH}_2\text{CO}_2\text{H}$                                                                                                                                                                                                                                                                                                                                                                                                                                                                                                          |
| Polyamino poly-carboxylic acids. | $-\text{COOH}$     | $-\text{NH}_2, =\text{NH}, \text{N}\equiv$ | $\begin{array}{c} \text{O} \quad \text{H} \\ \parallel \quad   \\ \text{C} - \text{O} - \text{N} = \\   \\ \text{OH} \end{array}$                                                                                                                                                                                                                                                                                                                                                                                                                                                                                                                                                                                                                                                                                   | $-\text{NH}_2, =\text{NH}, \text{N}\equiv, \text{COOH}$ | Uroanic acid<br>$\text{H}_2\text{NCOHN}-\text{C}(\text{NHCOHN})-\text{COOH}$<br><br>Kynurenone<br>$\text{H}_2\text{N}-\text{CH}_2-\text{C}=\text{CH}-\text{CH}(\text{NH}_2)\text{CO}_2\text{H}$<br><br>Ethylene diamine tetra acetic acid<br>$\text{HO}_2\text{CH}_2\text{C}(\text{H})-\text{N}(\text{H})-\text{C}(\text{H})-\text{N}(\text{H})-\text{C}(\text{H})-\text{CH}_2\text{CO}_2\text{H}$<br>$\begin{array}{c} \text{HO}_2\text{CH}_2\text{C} \quad \text{H} \quad \text{H} \quad \text{CH}_2\text{CO}_2\text{H} \\   \quad \quad \quad   \\ \text{N} - \text{C} - \text{C} - \text{N} \\   \quad \quad \quad   \\ \text{H} \quad \quad \quad \text{CH}_2\text{CO}_2\text{H} \end{array}$                                                                                                                                                                                                                              |

It should also be noted that, in addition to the proper functional groups, the compounds belonging to the aliphatic series do not have individual non-polar radicals any longer than 4 carbons.

As is well known, most of these aliphatic amino-acids are present (decomposition products of proteins) in the hydrolysis liquor of vegetal matters (soy-bean, wheat-, sugar cane-, beet juices, etc.) and can be extracted therefrom. Certain polyamino polycarboxylic acids are syn-

65 and marketed under the trade name "Nullapon B".

The preferred procedure for flotation of non-sulfide ores (so-called "non-metallics") is to add at first the organic gangue depressant, in 70 amounts of approximately 0.05 kg. per metric ton of ore, and to condition (agitate) for several minutes. Dispersants and pH regulators (sodium silicate, sodium carbonate, caustic, hydrofluosilic acid, sulfuric acid) are then fed as 75 usual, and finally the flotation is performed with

## 11

a properly selected collector such as a fatty acid emulsion. A frother may be added, if required. As the depressing effect of the organic compound is sufficiently strong, a paraffin oil (gas oil, kerosene, etc.) can be used in addition to the chemically active collector, reducing substantially the amount of the latter. This is a further advantage of the process.

In the following "schematic" tests, the collecting emulsion was chosen so as to be very unselective by itself, in order to emphasize the depressing action of the new reagents. This is evidently bad flotation practice, but a convenient experimental procedure. "Synthetic ores" (i. e. mixtures of more or less pure minerals) were used, and the flotation performed on 30-grs. samples in a small laboratory cell (capacity: 150 cc.), the dilution being 1:5 (distilled water).

Tests I to V were run with a -65 mesh mixture containing 10% malachite, 30% limestone and 60% quartz (3.77-3.80% Cu). The collecting emulsion had the following composition:

|                                                | cc.  |
|------------------------------------------------|------|
| Oleic acid                                     | 2.0  |
| Heavy mineral oil (paraffin oil)               | 1.5  |
| Kerosene                                       | 0.5  |
| 1% solution of sodium lauryl sulfate ("Dreft") | 3.0  |
| 3% solution of Emulsol XI                      | 2.0  |
| Water                                          | 21.0 |

## TEST I

## Reagents

|                                                     |                |
|-----------------------------------------------------|----------------|
| 0.1 cc. 10% soda ash solution                       | Condit. 4 min. |
| 0.2 cc. 10% vol. solution of sodium silicate 38° Bé |                |
| 1.0 cc. emulsion                                    | Condit. 2 min. |
| 1 droplet frother B-23 (Amer. Cyanamid Co.)         |                |
| 0.3 cc. emulsion                                    |                |

## Results

| Products    | Weight, grs. | Per cent Cu | Grs. Cu | Recov. per cent |
|-------------|--------------|-------------|---------|-----------------|
| Conc.       | 14.73        | 7.21        | 1.062   | 95.08           |
| Tails       | 14.84        | 0.37        | .055    |                 |
| Calc. heads | 29.57        | 3.78        | 1.117   |                 |

## Comments

The recovery is good, due to the strong collecting properties of the emulsion, but the grade of the concentrate is naturally low, as a result of its lack of selectivity. The limestone and fine quartz particles were floated.

## TEST II

## Reagents

|                                                                        |                |
|------------------------------------------------------------------------|----------------|
| 0.1 cc. 10% soda ash solution                                          | Condit. 4 min. |
| 0.2 cc. 10% vol. sodium silicate 38° Bé                                |                |
| 1.0 cc. emulsion                                                       | Condit. 2 min. |
| 0.15 cc. 1% solution "Nullapon B" (Ethylene diamine tetra acetic acid) | Condit. 3 min. |
| 1 droplet frother B-23                                                 |                |
| 0.3 cc. emulsion                                                       |                |

## Results

| Products    | Weight, grs. | Per cent Cu | Grs. Cu | Recov. per cent |
|-------------|--------------|-------------|---------|-----------------|
| Conc.       | 12.35        | 8.53        | 1.053   | 94.18           |
| Tails       | 17.23        | 0.38        | .065    |                 |
| Calc. heads | 29.58        | 3.78        | 1.118   |                 |

## 12

## Comments

The grade of concentrate is only slightly better than in the foregoing test, as the depressant was added after the collector, and therefore could not properly react.

## TEST III

## Reagents

|                                         |              |
|-----------------------------------------|--------------|
| 0.15 cc. 1% solution Nullapon B         | Cond. 3 min. |
| 0.1 cc. 10% soda ash solution           |              |
| 0.2 cc. 10% vol. sodium silicate 38° Bé | Cond. 4 min. |
| 1.0 cc. emulsion                        |              |
| 1 droplet frother B-23                  | Cond. 2 min. |
| 0.3 cc. emulsion                        |              |

## Results

| Products    | Weight, grs. | Per cent Cu | Grs. Cu | Recov. per cent |
|-------------|--------------|-------------|---------|-----------------|
| Conc.       | 4.31         | 24.92       | 1.074   | 95.89           |
| Tails       | 25.39        | 0.18        | .046    |                 |
| Calc. heads | 29.70        | 3.77        | 1.120   |                 |

## Comments

This test shows the high selectivity obtainable by the proper use of an organic complexing depressant. The grade of concentrate rose from 7.21% to 25%, while the tailings dropped from 0.37% to 0.18%.

## TEST IV

## Reagents

|                                         |              |
|-----------------------------------------|--------------|
| 0.15 cc. 1% solution glutamic acid      | Cond. 3 min. |
| 0.1 cc. 10% soda ash solution           |              |
| 0.2 cc. 10% vol. sodium silicate 38° Bé | Cond. 4 min. |
| 1.0 cc. emulsion                        |              |
| 1 droplet frother B-23                  | Cond. 2 min. |
| 0.3 cc. emulsion                        |              |

## Results

| Products    | Weight, grs. | Per cent Cu | Grs. Cu | Recov. per cent |
|-------------|--------------|-------------|---------|-----------------|
| Conc.       | 5.24         | 19.70       | 1.032   | 93.31           |
| Tails       | 23.35        | 0.31        | .074    |                 |
| Calc. heads | 29.09        | 3.80        | 1.106   |                 |

## Comments

The grade of concentrate is 19.70% versus 7.21; the tailings are slightly better than in Test I, due to the use of an organic complexing depressant.

## TEST V

## Reagents

|                                         |              |
|-----------------------------------------|--------------|
| 0.15 cc. 1% solution dl. Aspartic acid  | Cond. 3 min. |
| 0.1 cc. 10% soda ash solution           |              |
| 0.2 cc. 10% vol. sodium silicate 38° Bé | Cond. 4 min. |
| 1.0 cc. emulsion                        |              |
| 1 droplet frother B-23                  | Cond. 2 min. |
| 0.3 cc. emulsion                        |              |

## Results

| Products    | Weight, grs. | Per cent Cu | Grs. Cu | Recov. per cent |
|-------------|--------------|-------------|---------|-----------------|
| Conc.       | 7.61         | 13.80       | 1.050   | 94.45           |
| Tails       | 21.76        | 0.28        | .061    |                 |
| Calc. heads | 29.36        | 3.78        | 1.111   |                 |

13  
Comments

The grade of concentrate is 13.80 versus 7.21; better tailings are also obtained.

The next two tests were made with a -65 mesh mixture containing 5 gr. rhodochrosite (manganese carbonate) and 25 gr. of silica sand for each 30 gr. head sample.

## TEST VI

## Reagents

|                                                                         |              |
|-------------------------------------------------------------------------|--------------|
| 0.25 cc. 10% soda ash solution                                          | Cond. 4 min. |
| 0.10 cc. 10% vol. sodium silicate 38° Bé                                | Cond. 3 min. |
| 0.10 cc. 5% "monopolsoap" (sodium salt of highly sulfonated castor oil) | Cond. 2 min. |
| 0.05 cc. oleic acid                                                     |              |
| 0.03 cc. kerosene                                                       |              |
| 1 droplet frother B-23                                                  |              |

## Results

| Products     | Weight, grs. | Percent Mn | Grs. Mn | Recov. per cent |
|--------------|--------------|------------|---------|-----------------|
| Cone.        | 12.38        | 10.2       | 1.2627  | 94.06           |
| Tails.       | 17.14        | 0.63       | 0.0798  |                 |
| Calc. heads. | 29.52        | 4.54       | 1.3425  |                 |

## Comments

Good recovery, but the tailings are relatively high and the concentrate is contaminated with fine silica.

## TEST VII

## Reagents

|                                          |              |
|------------------------------------------|--------------|
| 0.1 cc. 1% solution of Nullapon B        | Cond. 3 min. |
| 0.25 cc. 10% soda ash solution           | Cond. 4 min. |
| 0.10 cc. 10% vol. sodium silicate 38° Bé | Cond. 3 min. |
| 0.10 cc. 5% "Monopolsoap"                |              |
| 0.05 cc. oleic acid                      |              |
| 0.03 cc. kerosene                        |              |
| 1 droplet frother B-23                   | Cond. 2 min. |

## Results

| Products     | Weight, grs. | Percent Mn | Grs. Mn | Recov. per cent |
|--------------|--------------|------------|---------|-----------------|
| Cone.        | 7.22         | 17.19      | 1.2411  | 94.55           |
| Tails.       | 22.37        | 0.32       | 0.0715  |                 |
| Calc. heads. | 29.59        | 4.44       | 1.3126  |                 |

## Comments

Higher grade of concentrate (17.19% versus 10.2%) and better tailings, due to the use of an organic complexing depressant.

The next test was run with a 30-gr. sample containing 22.5 grs. of a mixture of 65% silica and 35% limestone, 2.5 grs. chalcosite (with some

65 The results are tabulated below:

| Product  | Weight | Copper, per cent | Copper grs. | Rec., per cent | Ratio of cone, |
|----------|--------|------------------|-------------|----------------|----------------|
| 1st cone | 12.95  | 31.84            | 4.130       | 41.31          | 1:20.22        |
| 2nd cone | 18.40  | 17.54            | 3.230       | 32.31          | 1:11.14        |
| 3rd cone | 14.85  | 4.28             | 0.636       | 6.38           | 1: 2.72        |
| Tails    | 589.10 | 0.34             | 2.002       | 20.02          |                |
| Heads    | 635.30 | 1.57             | 9.998       | 100.00         |                |

chalcopyrite), and 5 grs. galena. In this case, an excess of the organic complexing depressant was added, in order to float selectively the lead sulfide from the copper mineral.

5

## TEST VIII

## Reagents

|                                         |              |
|-----------------------------------------|--------------|
| 1.0 cc. 1% solution of Glutamic acid    | Cond. 5 min. |
| 0.15 cc. 10% soda ash solution          |              |
| 0.1 cc. 10% vol. sodium silicate 38° Bé |              |
| 0.2 cc. 1% sodium ethyl xanthate        |              |
| 1 droplet frother B-23                  |              |

## Results

| Products    | Weight, grs. | Per cent Cu | Grs. Cu | Depress. per cent |
|-------------|--------------|-------------|---------|-------------------|
| Conc.       | 4.72         | 1.31        | 0.062   |                   |
| Tails       | 24.77        | 7.03        | 1.741   | 96.56             |
| Calc. heads | 29.49        | 6.114       | 1.803   |                   |

25 The following example will further illustrate how the said invention may be carried out in practice, but the invention is not restricted to this example.

30

A deslimed (+10 mu) oxide copper ore from Miami (Arizona) had been floated with ethyl xanthate, oleic acid, soda ash, sodium silicate and cyanide as specific depressant (following the Earl Fisher process). The results of the roughing operation were reported as follows by the operators:

35

| Product   | Weight | Copper, per cent | Copper grs. | Rec., per cent | Ratio of concen. |
|-----------|--------|------------------|-------------|----------------|------------------|
| 1st conc. | 13.9   | 7.1              | 0.9869      | 66.00          | 1:4.7            |
| 2nd conc. | 14.7   | 1.2              | 0.1764      | 11.80          | 1:0.8            |
| 3rd conc. | 18.5   | 0.65             | 0.1203      | 8.05           |                  |
| Tails     | 52.9   | 0.40             | 0.2116      | 14.15          |                  |
| Heads     | 100.0  | 1.50             | 1.4952      | 100.00         |                  |

50 The same ore was floated without cyanide, but with an added amount of ethylene diamine tetra acetic acid ("Nullapon B") as follows:

1000 grs. ore -65 mesh were deslimed at 10 microns, yielding 670 grs. of a sand product with 1.575% Cu. These sands were floated as follows in a laboratory Fagergreen cell:

55

|                                            |              |
|--------------------------------------------|--------------|
| Nullapon B, 2% solution, 1.0 cc            | Cond. 3 min. |
| Soda ash, 10% solution, 2.0 cc             |              |
| Silicate 38° Bé, 10% vol., 1.0 cc          |              |
| Sodium ethyl xanthate, 1% solution, 1.5 cc |              |
| Alkanol S. A., 1% (emulsifier), 0.5 cc     |              |
| Oleic acid, 0.3 cc                         |              |
| Paraffin oil, 0.1 cc                       |              |
| Kerosene, 0.1 cc                           |              |

60

The results are tabulated below:

15

The 3rd concentrate can be considered as a middling, and the distribution of the copper in the recovery may be figured as 4.6% in the concentrate and 1.0% in the tails, thus raising the final recovery to 78.2%.

While in the "normal" flotation a concentrate with 7.1% Cu (Rec. 66.0%) is obtained, the ratio being 1:4.7, the flotation following the present invention yields a product with 23.5% Cu (Rec. 73.6%). The tailings are 0.46 versus 0.34, and 10 the middlings of the operation first reported are lower than the heads.

Comparison of these results shows that the ratio of concentration is considerably raised by 15 conditioning the pulp with a polyamino poly-carboxylic acid.

Therefore, the use, according to the present invention, of organic reagents accomplishing the purpose of gangue depression through complexing detrimental cations into a water soluble or 20 hydrophilic chelate compound constitutes a marked advance in the art of froth flotation, and is highly advantageous in improving the selectivity of the collectors, thus improving the grade of concentrate.

What is claimed is:

1. In the concentration by froth flotation of non-sulfide ores, which includes the subjecting of such material when finely ground to flotation in the presence of an emulsion of mineral oil and fatty acid stabilized by a wetting agent as 30 collector and by the addition of usual modifiers, the step of adding first to the pulp an amount of the order of 0.05 kg. per metric ton of a non-collecting organic compound containing one 35 amino nitrogen in alpha or beta (1 or 2) position to one carboxyl group and having the following general schematic formula:



16

where R is a substituted organic aliphatic, aromatic or heterocyclic radical with at least one carboxyl group or one amino nitrogen; said organic compound being adapted to react with the gangue activating cations of the pulp to yield a water soluble or hydrophilic chelate compound having the schematic general formula:



where Me is a metal atom (monovalent) replacing the hydrogen of the carboxyl group by electron exchange and linked to the negative amino nitrogen by the coordination bond (dative bond), while the free carboxyl- or amino-function or functions attached to R are imparting water solubility to the chelate compounds.

2. The process as claimed in claim 1, where the depressing organic compounds are polyvalent amino acids extracted from protein-rich natural hydrolytes.

3. The process as claimed in claim 1, where the depressing organic compounds are polyvalent amino acids extracted from protein-rich natural hydrolytes.

4. The process as claimed in claim 1, where the depressing organic compound is a polyamino polycarboxylic acid corresponding to the general formula:



where R is a lower alkylene radical and Ac the radical of an aliphatic organic acid with less than 9 carbon atoms in the chain.

GREGOIRE GUTZEIT.